

## UNITED STATES PATENT OFFICE

1,932,871

## ALUMINUM ALLOYS

Robert T. Wood, Cleveland, Ohio, assignor to  
Aluminum Company of America, Pittsburgh,  
Pa., a corporation of Pennsylvania

No Drawing. Continuation of application Serial  
No. 634,155, September, 21, 1932. This applica-  
tion November 30, 1932. Serial No. 645,125

## 1 Claim. (Cl. 75—1)

This invention relates to aluminum base al-  
loys containing magnesium. The invention has  
for its object the improvement of alloys of this  
class by the addition thereto of about 0.05 to  
5 2.0 per cent by weight of calcium. The invention  
is particularly concerned with the specific  
alloys hereinafter described.

This application is a continuation of my co-  
pending application Serial No. 634,155 which is,  
10 in part, a continuation of my copending applica-  
tion Serial No. 595,231. Inventions disclosed  
but not claimed herein are claimed in my co-  
pending applications Serial Nos. 595,231, filed  
February 25, 1932, and 645,108 to 645,124 in-  
15 clusive, all filed November 30, 1932.

Considerable difficulty has heretofore been en-  
countered in attempts to commercially produce  
castings of aluminum base alloys containing sub-  
stantial amounts of magnesium. This difficulty  
20 is encountered both in the making of sand cast-  
ings and permanent mold or chill-mold castings,  
although the nature of the difficulty differs some-  
what in each case. In the case of sand cast-  
ings there occurs a reaction between the molten  
25 aluminum base alloy containing magnesium and  
the ordinary sand-mold materials, or vapors gen-  
erated therefrom. There is also a reaction with  
the atmosphere. In addition, the magnesium-  
containing aluminum base alloy does not flow  
30 freely through narrow mold sections at ordinary  
pouring temperatures and, if the pouring tem-  
perature be raised, the solidified alloy is un-  
sound. If the aluminum base alloy containing  
magnesium be cast in a chill-mold the reaction  
35 effect is minimized to some extent, but the trou-  
bles arising from cold-shuts and mis-runs are  
accentuated because of the more rapid chilling  
of the molten metal. The considerations ap-  
ply to the aluminum base alloys specifically dis-  
40 closed herein and particularly to such alloys.

I have discovered that when calcium is added  
to aluminum base alloys of the type and com-  
position herein described, these difficulties are,  
45 to a considerable extent, eliminated. The cal-  
cium should be present in amounts ranging from  
0.05 per cent to 2.0 per cent by weight subject  
to specific considerations as hereinafter dis-  
closed.

In the melting of aluminum alloys of the  
50 compositions herein described, a viscous scum  
often forms at the surface of the molten metal.  
Failure of the molten metal to run properly  
through narrow mold apertures is caused, in  
part, by shreds or particles of this scum being  
55 suspended in the molten metal and offering a

resistance to the free passage of the metal  
through the apertures. Regardless of the cause  
of this low fluidity, I have discovered that the  
addition to the alloy of relatively small amounts  
of calcium, in the preferred range between 0.05 60  
to 0.5 per cent, improves the casting character-  
istics to a very considerable extent and sim-  
ultaneously effects a reduction of the scum or dross  
collecting at or near the surface. In the casting  
of articles in sand molds, I prefer to add cal-  
cium in amounts less than about 0.5 per cent  
except in instances where some reduction of  
tensile strength or other mechanical or tensile  
property is immaterial. In amounts of more  
than 0.5 per cent the calcium addition produces 70  
the advantages enumerated herein but has a  
tendency to lower some of the physical proper-  
ties of the alloys. This effect is not harmful  
when calcium is present in amounts of about  
0.5 per cent or less, but when high strength is 75  
not a desideratum the calcium may be used in  
amounts up to about 2.0 per cent. In intricate  
permanent mold castings, where casting trou-  
bles are very serious if no calcium be added, the  
improved physical properties obtained coincident 80  
with the production of good castings more than  
offset the diminution in properties which might  
otherwise result from the use of the calcium.

I have also discovered that when calcium is  
added to aluminum base alloys containing mag- 85  
nesium, the amount of gas evolved during solidi-  
fication of the alloys is considerably reduced.  
When from about 0.05 per cent to 2.0 per cent  
by weight of calcium is added to the alloys, the  
amount of gas evolved becomes less marked with 90  
increasing calcium content and the reduction of  
gas evolution may be so marked that the molten  
metal cools to the solidification temperature  
with a smooth mirror-like surface. I prefer to  
restrict the amount of calcium added to 2.0 per 95  
cent or less since above this amount the physical  
properties of the alloys may be too seriously af-  
fected. If the best physical properties are de-  
sired with an improved, although not complete,  
degree of gas prevention, I keep the calcium 100  
content of the alloys between 0.05 per cent and  
about 0.5 per cent.

In the application of the principles of my in-  
vention I have determined that certain alum-  
inum base alloys containing magnesium are par- 105  
ticularly benefited thereby. For example, a very  
useful aluminum base alloy is one containing  
about 2.0 to 9.0 per cent of magnesium and 0.05  
per cent to 2.0 per cent of calcium, as is also  
aluminum base alloy containing about 2.0 to 15.0 110

per cent of magnesium, 0.1 to 3.5 per cent of cobalt, and 0.05 to 2.0 per cent of calcium to which other elements such as copper, antimony, bismuth, nickel, manganese, and other well known alloying elements may be added to produce particular properties therein.

Likewise is the addition of 0.05 to 2.0 per cent of calcium beneficial to those aluminum base alloys which contain about 2.0 to 15.0 per cent of magnesium and 0.05 to 0.4 per cent of at least one of the class of metals here defined as antimony and bismuth, such alloys being very useful where use at high temperatures is contemplated. Calcium may likewise be added to improve such alloys when they contain, in addition to magnesium and antimony and/or bismuth, one or more of such alloying elements as cobalt, copper, nickel, manganese, zinc, etc. which may be added to modify or produce a specific property in the alloy.

The addition of 0.05 to 2.0 per cent of calcium is very beneficial in the case of a series of aluminum base alloys which contain as major alloying elements about 2.0 to 10.0 per cent of magnesium and about 0.2 to 5.0 per cent of nickel. For instance, an aluminum base alloy containing 3.0 to 7.5 per cent of magnesium and 0.2 to 2.0 per cent of nickel is improved by the addition of 0.05 to 2.0 per cent of calcium as is, likewise, this same alloy when it also contains about 0.05 to 0.4 per cent of one or more of the class of elements composed of antimony and bismuth. Another excellent aluminum base alloy prepared in accordance with the principles of my invention is one containing 3.0 to 8.0 per cent of magnesium, 0.5 to 4.0 per cent of nickel, 0.5 to 4.0 per cent of manganese, and 0.05 to 2.0 per cent of calcium, which alloy may also be improved, particularly for application at high temperatures, by the addition of 0.05 to 0.4 per cent of at least one of the class of elements composed of antimony and bismuth.

The principles of my invention find particular application in the case of aluminum base alloys containing magnesium, nickel, and chromium, and aluminum base alloys containing magnesium, nickel, and copper, as well as those alloys containing magnesium, nickel, and cobalt. Examples may be given of aluminum base alloys containing 2.0 to 10.0 per cent of magnesium, 0.2 to 5.0 per cent of nickel, 0.5 to 3.5 per cent of chromium, and 0.5 to 2.0 per cent of calcium. An aluminum base alloy containing 3.0 to 8.0 per cent of magnesium, 0.5 to 3.5 per cent of nickel, 0.5 to 3.5 per cent of chromium, and 0.05 to 2.0 per cent of calcium has excellent casting properties and the high temperature properties of this alloy can be favorably affected by the addition of 0.05 to 0.4 per cent of at least one of a

class of elements composed of bismuth and antimony. Examples may be given of aluminum base alloy containing 2.0 to 10.0 per cent of magnesium, 0.2 to 5.0 per cent of nickel, 1.0 to 6.0 per cent of copper, and 0.05 to 2.0 per cent of calcium. An excellent alloy of this type is one containing 3.0 to 8.0 per cent of magnesium, 0.5 to 5.0 per cent of nickel, 1.0 to 6.0 per cent of copper, and 0.05 to 2.0 per cent of calcium with or without 0.05 to 0.4 per cent of at least one of the class of elements composed of antimony and bismuth and with or without the further addition of 0.5 to 3.5 per cent of at least one of a class of elements composed of cobalt and chromium, and with or without the further addition of 0.1 to 1.0 per cent of at least one of a class of elements composed of tungsten, vanadium, molybdenum, titanium, and zirconium.

Other excellent alloys are those aluminum base alloys containing about 2.0 to 10.0 per cent magnesium, 0.2 to 5.0 per cent nickel, 0.1 to 3.5 per cent cobalt, and 0.05 to 2.0 per cent of calcium. A particular example of this class of alloys, which may also contain with considerable advantage 0.05 to 0.4 per cent of a class of elements composed of antimony and bismuth, is the aluminum base alloy containing 3.0 to 8.0 per cent magnesium, 0.5 to 4.0 per cent nickel, 0.1 to 3.0 per cent cobalt, and 0.05 to 2.0 per cent calcium.

Among other magnesium-containing aluminum base alloys which I have found to be particularly benefited by the presence of calcium are numbered the aluminum base alloys containing 3.0 to 8.0 per cent of magnesium, 1.0 to 6.0 per cent of copper, 0.5 to 3.5 per cent of chromium, and 0.05 to 2.0 per cent of calcium, with or without the addition of 0.05 to 0.4 per cent of at least one of a class of metals composed of antimony and bismuth and with or without the addition of other alloying elements.

The alloys herein described may be produced by the usual methods of alloying metals. The calcium is preferably added to the molten alloy by thrusting the calcium beneath the surface with tongs or other suitable instrument. The aluminum used in preparing the alloys may be pure or it may contain the impurities found in commercial grades of this metal. Ordinarily a good commercial grade of virgin aluminum will give excellent results and is preferable.

Having thus explained and described my invention, I claim:

A metallic alloy consisting of about 2 to 15 per cent by weight of magnesium, 0.1 to 3.5 per cent by weight of cobalt, and 0.05 to 2.0 per cent by weight of calcium, the balance being aluminum.

ROBERT T. WOOD.

135

60

140

65

145

70

150

75